

## 1

3,649,612

TREATMENT OF ROSIN WITH AN ARYL THIOL  
 Roland Pierre Franz Scharrer, Pelham, N.Y., assignor to  
 Arizona Chemical Company, New York, N.Y.  
 No Drawing. Continuation-in-part of application Ser. No.  
 827,174, May 23, 1969. This application Apr. 20, 1970,  
 Ser. No. 30,233

Int. Cl. C09f 1/04

U.S. CL. 260—98

8 Claims

## ABSTRACT OF THE DISCLOSURE

Rosin is disproportionated and bleached by heating at temperatures of about 180–350° C., and for a time sufficient to reduce the abietic acid content to less than 15%, in the presence of 0.01–1% of an arylthiol.

This application is a continuation-in-part of copending application Ser. No. 827,174, filed May 23, 1969, now abandoned.

This invention relates to the simultaneous bleaching and disproportionation of rosin.

The term rosin, as used herein, includes tall oil rosin, wood rosin, gum rosin, crude materials and mixtures containing any of the foregoing, and, in general, any materials containing abietic acid, including tall oil fractions containing various proportions of rosin and fatty acids.

Rosin soap is a preferred emulsifier in rubber polymerization processes. In this application particularly, it is important that the rosin to be used first be stabilized, i.e. rendered less sensitive to oxidation, by conversion of most of the conjugated rosin acids as typified by abietic acid contained therein to an isomer without conjugated double bonds, such as, for example, dehydroabietic acid. This is commonly done by "disproportionation," a term used in the art to describe displacement of hydrogen atoms in the abietic acid molecule.

It is known in the art that rosin can be disproportionated by heating it at elevated temperature in the presence of catalysts. Typically, U.S. Pat. 3,277,072 (Patrick and Bestul) teaches the use of iodine, while others (U.S. Pats. 2,130,997; 2,239,555; 2,138,183; 2,154,629; 2,486,183 and 2,580,496) teach the use of noble metals, such as platinum or palladium. U.S. Pats. 2,503,268 and 2,497,882 suggest the use of sulfur or selenium. These treatments, however, result only in disproportionation. The treated rosin not only is not bleached, but may actually darken as the result of heating for prolonged periods at high temperatures. Furthermore, additional expenses are inherent in these processes; substantial quantities of additive are required except in the case of the noble metal catalysts and their use, in turn, leads to loss of rosin during filtration. More recently, McBride and Wheelus U.S. Pat. 3,377,334 teaches disproportionation and bleaching by use of hydroxylated arylsulfides. While the catalysts of U.S. Pat. 3,377,334 suit their purpose admirably, their preparation is fairly difficult and comprises many steps.

It is an object of this invention to provide a process for the disproportionation and bleaching of rosin. It is a further object to provide a process not requiring removal of the disproportionating and bleaching agent from the treated rosin. Another object is to provide a class of treating agents having a high degree of activity, yet being readily and economically prepared. Yet another object is to provide rosin having a substantially reduced content of conjugated unsaturated acids of the non-benzenoid type, particularly abietic acid. A further object still is to provide treating agents which will not only dispropor-

## 2

tionate rosin, but will also markedly lower the softening point of the product.

These and other objects, features, and advantages of this invention will become apparent as the description thereof proceeds.

In accordance with the present invention, it has now been found that these objects can be achieved by a disproportionation process which comprises heating rosin in the presence of a small but effective amount of a particular treating agent.

The treating agents are aryl thiols which may be represented by the general formula:



where:

A represents an aromatic hydrocarbon nucleus including mono- and polycyclic aromatic hydrocarbons;

x is an integer from 0 to 3;

y is an integer from 1 to 3;

z is an integer from 0 to 3;

where the sum of x, y and z is not greater than 6 for monocyclic aromatics; and advantageously, polycyclic aromatic hydrocarbons may be used having up to about 18 carbon atoms in the aromatic rings. However, the invention need not be confined to these.

R is a hydrocarbon group, e.g. alkyl, cycloalkyl, and aryl, or suitable substituted alkyl, cycloalkyl, and aryl R desirably contains from 1 to 22 carbon atoms inclusive. Preferred alkyl groups are those containing up to 8 carbon atoms inclusive. Preferred aryl groups are those containing 6 to 18 carbon atoms inclusive, typically phenyl, naphthyl, and anthracyl. Typical cycloalkyl groups contain 3 to 8 carbon atoms in the ring, e.g. cyclopropyl, cyclopentyl, cyclohexyl. Alternatively R

40 may also be a carboxylic acid, halogen, nitro, or amino group.



The terms "treating agent" or "disproportionating agents," as used herein, are defined by Formulas I and II above.

Typical and non-limiting examples of such treating agents are the following:

2-hydroxy-1-mercaptophenyl

2,4-dihydroxythiophenol

Toluene-3,4-dithiol

Thiosalicylic acid

4-nonyl-1,2-benzenedithiol

4-chlorothiophenol

Thiophenol

2-aminothiophenol

4-aminothiophenol

4-bromothiophenol

4-tertiarybutylthiophenol

4-nitrothiophenol

Ortho-thiocresol

Meta-thiocresol

Para-thiocresol

The conditions for disproportionation and bleaching will vary depending on the starting rosin material and the degree of disproportionation desired. Tall oil rosin is effectively disproportionated by heating the rosin in the presence of the treating compound at from about 180° C. to 350° C. for from about 1 to 8 hours, wherein the longer times correspond to lower treating temperature and vice versa. Preferred ranges are from about 250° C. to 300° C. for from about 3 to 6 hours.

The degree of disproportionation may be controlled as desired and as dictated by the degree of stability required in the end use. Generally, the abietic acid content should be reduced to less than about 15% by weight of the rosin and preferably to the more commercially acceptable level of less than about 5%, same basis. Reduction of abietic acid content can be followed during the reaction by sampling and analysis, employing any of the procedures known in the art such as the "Rubber Reserve" (ultraviolet) method (as disclosed in U.S. Pat. No. 3,377,334) or, preferably by gas-liquid chromatography.

Sequence of admixture of the rosin or rosin mixture with the treating agent is not critical. Likewise, the rosin may be heated to the desired temperature before the treating compound is added or rosin and additive may be first admixed, followed by heating. The process may be conducted at atmospheric, subatmospheric or superatmospheric pressures with corresponding variation in temperature and time of reaction. Also, the process may be carried out on batch, semi-continuous, or continuous basis. The disproportionation is ordinarily conducted under a blanket of inert gas, such as nitrogen, carbon dioxide, steam, and the like.

The following examples further illustrate the invention but are not limitative thereof except as indicated in the appended claims.

#### EXAMPLE I

To compare the disproportionation activity of three substituted arylthiols, the following experiments were carried out in sealed vessels under identical conditions. The rosin used was tall oil rosin conforming to the Naval Stores Act (Feb. 8, 1952) and Federal Specification LLL-R-6266, Class C (May 27, 1957), except for less bottoms content.

Rosin, 100 parts, water, 3 parts, and treating agent, 0.1, all parts by weight, were charged to the reaction vessel which was then sealed and heated at 290° C. for

active treating agent of this invention. Tall oil rosin, 500 parts, was charged to a glass reactor fitted with stirrer, thermometer, and inert gas inlet. 2,4-dihydroxythiophenol, 1 part, was added, and the mixture was heated under steam for five hours at 275° C. Samples were withdrawn at 0, 1, 3, and 5 hours and analyzed.

The results so obtained are shown in Table II. They show that disproportionation is substantially complete after 3 hours.

#### EXAMPLE III

To show that a catalyst of the type described by the present invention is effective in disproportionating and bleaching various types of rosin, tall oil rosin, as defined hereinbefore, wood rosin, and gum rosin were treated as in Example II above, using 2-hydroxy-1-naphthalenethiol as the disproportionating agent. The results are shown in Table III. This table shows that the compounds of the present invention are effective without regard to the type of rosin used. Analyses were carried out by gas-liquid chromatography.

#### EXAMPLE IV

To demonstrate the efficiency of a thiophenol in catalyzing disproportionation at temperatures lower than 290-320° C., 2-hydroxy-1-naphthalenethiol was used to disproportionate a standard rosin at 225° C. The gradual loss of abietic acid and the formation of dehydroabietic acid is listed below as observed at regular intervals. The lack of decarboxylation is noted by the constant acid number. See Table IV.

TABLE I

| Treating agent               | Abietic acid, percent | Dehydro-abietic acid, percent | Color | Softening point, <sup>1</sup> degrees |
|------------------------------|-----------------------|-------------------------------|-------|---------------------------------------|
| Toluene-3,4-dithiol-----     | 4.8                   | 44.2                          | WG    | 67.0                                  |
| Thiosalicylic acid-----      | 6.1                   | 40.7                          | WG    | 64.5                                  |
| 2,4-dihydroxythiophenol----- | 0.6                   | 46.0                          | K     | 61.0                                  |
| Feed (for comparison)-----   | 33.6                  | 21.2                          | N     | 81.0                                  |

<sup>1</sup> Ring and Ball Softening Point.

TABLE II

| Sample, hours | Abietic acid, percent | Dehydro-abietic acid, percent | Color | Acid Number |
|---------------|-----------------------|-------------------------------|-------|-------------|
| 0-----        | 34.7                  | 21.9                          | N     | 171         |
| 1-----        | 13.2                  | 34.1                          | X     | 167         |
| 3-----        | 3.8                   | 41.0                          | X     | 164         |
| 5-----        | 1.2                   | 44.5                          | WG    | 164         |

TABLE III

| Temp., °C.          | Treating agent, percent | Time, hours | Abietic acid, percent | Dehydro-abietic acid, percent | Color |
|---------------------|-------------------------|-------------|-----------------------|-------------------------------|-------|
| Tall oil rosin----- | 290                     | 0           | 34.7                  | 21.4                          | N     |
|                     |                         | 1           | 6.2                   | 36.3                          | X     |
|                     |                         | 2           | 2.3                   | 41.7                          | X     |
|                     |                         | 5           | 0.3                   | 43.3                          | WG    |
| Wood rosin-----     | 300                     | 0           | 39.6                  | 7.9                           | M     |
|                     |                         | 1           | 4.8                   | 39.8                          | X     |
|                     |                         | 3           | 1.3                   | 44.1                          | WW-X  |
|                     |                         | 5           | 0.8                   | 44.8                          | WG-N  |
| Gum rosin-----      | 300                     | 0           | 25.0                  | 6.0                           | K     |
|                     |                         | 1           | 5.6                   | 41.3                          | WG    |
|                     |                         | 3           | 2.1                   | 43.8                          | WG-N  |
|                     |                         | 5           | 0.7                   | 45.4                          | N     |

three hours. It was then cooled and opened, and the product was removed and analyzed. The data so obtained are shown in Table I. They show effective disproportionation. Abietic and dehydroabietic acid content was determined by gas-liquid chromatography. The colors are based on the conventional U.S. Department of Agriculture rosin scale.

#### EXAMPLE II

The purpose of this experiment was to demonstrate the progressive disproportionation of rosin by means of an

| Feed-----     | Abietic acid, percent | Dehydro-abietic acid, percent | Acid number |
|---------------|-----------------------|-------------------------------|-------------|
| Time (hours): |                       |                               |             |
| 1.0-----      | 16.8                  | 26.7                          | 171.5       |
| 3.0-----      | 6.5                   | 29.6                          | 171.8       |
| 5.0-----      | 2.4                   | 32.2                          | 170.6       |
| 7.0-----      | 0.9                   | 33.5                          | 171.8       |

The softness of the final rosin was noted by its ring and ball softening point of 57° C. The feed rosin had a ring and ball softening point of 81° C.

## EXAMPLE V

To demonstrate and compare the catalytic activity of two substituted thiophenols of the present invention versus that of 4,4'-thiobis(resorcinol), as used in U.S. Pat. No. 3,377,334, the following catalysts were employed with a standard rosin in sealed reaction vessels, in 0.1% concentration at 290° C. for 2.0 hours (gas-liquid chromatography analyses were carried out on the treated rosin). The results are shown in Table V.

TABLE V

|                              | Abietic acid, percent | Dehydro-abietic acid, percent | Softening point, <sup>1</sup> degrees |
|------------------------------|-----------------------|-------------------------------|---------------------------------------|
| Feed                         | 34.0                  | 21.4                          | 81                                    |
| 4,4'-thiobis(resorcinol)     | 4.2                   | 42.9                          | 64                                    |
| 2,4-dihydroxythiophenol      | 2.0                   | 42.2                          | 60                                    |
| 2-hydroxy-1-naphthalenethiol | 2.3                   | 41.7                          | 58                                    |

<sup>1</sup> Ring and Ball Softening Point.

## EXAMPLE VI

This example demonstrates the effective disproportionation of a mixture containing rosin. This mixture contained 55 parts of a tall oil fraction of typical analysis—94.2% fatty acids, 4.2% rosin acids, 1.6% unsaponifiables, and 45 parts of the same type rosin described in previous examples. The reaction temperature was 300° C., with 0.2% 2-hydroxy-1-naphthalenethiol employed. Treatment was carried out in an open vessel under a cover of steam. Rapid disproportionation was effected. Analyses were carried out by gas-liquid chromatography. The results are shown in Table VII.

TABLE VII

| Analysis                     | Feed | Hours |      |      |
|------------------------------|------|-------|------|------|
|                              |      | 1.0   | 3.0  | 5.0  |
| Oleic Acid, percent          | 23.2 | 32.4  | 33.7 | 34.1 |
| Linoleic acid:               |      |       |      |      |
| Conjugated, percent          | 7.4  | 11.3  | 10.7 | 9.2  |
| Non-conjugated, percent      | 21.2 | 5.8   | 3.9  | 2.8  |
| Abietic acid, percent        | 15.4 | 0.3   | 0.4  | 0.3  |
| Dehydroabietic acid, percent | 9.8  | 23.9  | 23.5 | 23.9 |

What is claimed is:

1. A method of treating a rosin which comprises heating said rosin at a temperature of from about 180° C.

to 350° C. in the presence of from about 0.01% to 1% by weight of said rosin of an arylthiol compound of the formula:



5

10 wherein:

- A represents an aromatic hydrocarbon group;  
 $x$  is an integer from 0 to 3;  
 $y$  is an integer from 1 to 3;  
 $z$  is an integer from 0 to 3; the sum of said  $x$ ,  $y$  and  $z$  being not greater than 6; and  
R is selected from the group consisting of a hydrocarbon group having from 1 to 22 carbon atoms, a carboxylic acid group, a halogen, a nitro group, and amino group.
2. The method of claim 1 wherein said R is an alkyl group with up to 8 carbon atoms.
  3. The method of claim 1 wherein said R is an aryl group with 6 to 18 carbon atoms.
  4. The method of claim 1 wherein said R is a cycloalkyl group with from about 3 to 8 carbon atoms.
  5. The method of claim 1 wherein said arylthiol is 2-hydroxy-1-naphthalenethiol.
  6. The method of claim 1 wherein said arylthiol is toluene-3,4-dithiol.
  7. The method of claim 1 wherein said arylthiol is thiosalicylic acid.
  8. The method of claim 1 wherein said arylthiol is 2,4-dihydroxythiophenol.

25

## References Cited

## UNITED STATES PATENTS

|           |         |                |          |
|-----------|---------|----------------|----------|
| 3,277,072 | 10/1966 | Patrick et al. | 260—97.5 |
| 3,377,334 | 4/1968  | McBride et al. | 260—98   |
| 3,417,071 | 12/1968 | Wheelus        | 260—108  |
| 3,423,389 | 1/1969  | Wheelus        | 260—97.5 |

DONALD E. CZAJA, Primary Examiner

R. W. GRIFFIN, Assistant Examiner

U.S. CL. X.R.

260—97.5; 108

40

45